

## 1

3,674,481

### IMAGE RECEIVING MATERIAL FOR THE SILVER SALT DIFFUSION PROCESS

Anita von Konig and Werner Liebe, Leverkusen, and Helmut Timmler, Wuppertal-Vohwinkel, Germany, assignors to Agfa-Gevaert Aktiengesellschaft, Leverkusen, Germany

No Drawing. Filed May 27, 1970, Ser. No. 41,085  
Claims priority, application Germany, June 14, 1970,  
P 19 30 339.0  
Int. Cl. G03c 5/54

U.S. Cl. 96—29

2 Claims

#### ABSTRACT OF THE DISCLOSURE

A light-insensitive image receiving material for the silver salt diffusion process comprising an image receiving layer which contains a compound of the mercapto triazole series.

The invention relates to an image receiving material for the silver salt diffusion process which contains heterocyclic dimercapto compounds for improving the stability of the finished silver images.

The silver salt diffusion process for the direct production of positives is described in French Pat. No. 879,995. In this process, the unexposed and undeveloped silver halide of an exposed silver halide emulsion layer is dissolved during development, and transferred to an image receiving layer, which is in close contact with the exposed silver halide emulsion layer, so as to produce a positive image in the image receiving layer upon development of the transferred silver halide in the presence of development nuclei which are uniformly distributed in the image receiving layer. The terms negative and positive are to be understood as being only in relation to one another, i.e. direct negatives can also be obtained from a negative original by the same process.

The complex forming agent required for dissolving the unexposed and undeveloped silver halide, particularly sodium thiosulfate, is added either to the developer or to the image receiving layer. The finished copy, therefore, still contains thiosulfate in quantities of about 0.5 to 1.5 g./m.<sup>2</sup>. The presence of compounds which form complexes with the silver salt gives rise to the disadvantages that these complex forming agents reduce the concentration of silver ions and thereby facilitate the oxidation of the metallic silver. The image silver is, therefore, easily attacked by oxidation and converted into a complex or simple silver salt. This causes particularly in a moist atmosphere fading of the silver image or a brown discoloration of the silver in the image. The image silver disappears particularly readily in those areas where only a little silver was deposited on the copies because of short contact times. In practice, contact times of about 5 to 15 seconds have recently become customary so that only a little silver is deposited, the stability of which is, therefore, reduced in the presence of sodium thiosulfate.

It is among the objects of the invention to modify the silver salt diffusion process so that the silver images obtained will have improved stability.

We now have found an image receiving material for the silver salt diffusion process which comprises an image receiving layer which may contain development nuclei, the image receiving layer containing a mercapto triazole derivative of the following formula:

## 2



5 in which

R<sup>1</sup>=a mercapto group or the group



10 R<sup>2</sup>=(I) an amino group or a substituted amino group, (II) together with R<sup>1</sup> the ring members required for completing a 2-mercaptothiodiazole ring or (III) in the case of a bis-triazole compound, R<sub>2</sub>=R<sub>3</sub>;

15 R<sup>3</sup>=hydrogen; alkyl containing up to 8 C-atoms, preferably containing 1 to 3 C-atoms; aryl preferably a radical of the phenyl or naphthyl series; aralkyl such as benzyl or phenylethyl; cycloalkyl such as cyclohexyl; or an amino group; the radicals, in particular phenyl rings, may be substituted, e.g. with halogen atoms such as chlorine or bromine; or alkyl or alkoxy groups containing preferably up to 5 C-atoms, or hydroxyl groups; 20 Y=an alkylene chain containing 3 to 10 methylene groups which are interrupted by hetero atoms such as oxygen or sulfur or imino groups.

25 Suitable compounds are summarized below:

| Compound | Compounds in which—                 |                                                                    | Melting point, °C. |
|----------|-------------------------------------|--------------------------------------------------------------------|--------------------|
|          | R <sup>3</sup>                      | Y                                                                  |                    |
| 1        | C <sub>6</sub> H <sub>5</sub>       | CH <sub>2</sub> —O—CH <sub>2</sub>                                 | 275                |
| 2        | NH <sub>2</sub>                     | CH <sub>2</sub> —O—CH <sub>2</sub>                                 | 219                |
| 3        | 35                                  | CH <sub>2</sub> —O—CH <sub>2</sub>                                 | 253                |
|          |                                     |                                                                    |                    |
| 4        | 40                                  | H                                                                  | 310                |
| 5        | CH <sub>2</sub> =CH—CH <sub>2</sub> | CH <sub>2</sub> —S—CH <sub>2</sub>                                 | 178                |
| 6        | C <sub>6</sub> H <sub>5</sub>       | CH <sub>2</sub> —S—CH <sub>2</sub>                                 | 304                |
| 7        | NH <sub>2</sub>                     | CH <sub>2</sub> —S—CH <sub>2</sub>                                 | 251                |
| 8        | CH <sub>3</sub>                     | CH <sub>2</sub> —S—CH <sub>2</sub>                                 | 265                |
| 9        | CH <sub>3</sub>                     | (CH <sub>2</sub> ) <sub>2</sub> —S—(CH <sub>2</sub> ) <sub>2</sub> | 225                |
| 10       | NH <sub>2</sub>                     | (CH <sub>2</sub> ) <sub>2</sub> —S—(CH <sub>2</sub> ) <sub>2</sub> | 225                |
| 11       | CH <sub>2</sub> —CH=CH <sub>2</sub> | (CH <sub>2</sub> ) <sub>2</sub> —S—(CH <sub>2</sub> ) <sub>2</sub> | 192                |
| 12       | C <sub>6</sub> H <sub>5</sub>       | (CH <sub>2</sub> ) <sub>2</sub> —S—(CH <sub>2</sub> ) <sub>2</sub> | 253                |
| 13       | H                                   | (CH <sub>2</sub> ) <sub>2</sub> —S—(CH <sub>2</sub> ) <sub>2</sub> | 281                |
| 14       | H                                   | CH <sub>2</sub> —S—CH <sub>2</sub> —S—CH <sub>2</sub>              | 288                |
| 15       | CH <sub>2</sub> —CH=CH <sub>2</sub> | CH <sub>2</sub> —S—CH <sub>2</sub> —S—CH <sub>2</sub>              | 141                |
| 16       | CH <sub>3</sub>                     | CH <sub>2</sub> —S—CH <sub>2</sub> —S—CH <sub>2</sub>              | 248                |
| 17       | C <sub>6</sub> H <sub>5</sub>       | CH <sub>2</sub> —S—CH <sub>2</sub> —S—CH <sub>2</sub>              | 268                |
| 18       | NH <sub>2</sub>                     | CH <sub>2</sub> —S—CH <sub>2</sub> —S—CH <sub>2</sub>              | 210                |
| 19       | H                                   | (CH <sub>2</sub> ) <sub>2</sub> —S—(CH <sub>2</sub> ) <sub>3</sub> | 248                |
| 20       | CH <sub>3</sub>                     | (CH <sub>2</sub> ) <sub>2</sub> —S—(CH <sub>2</sub> ) <sub>3</sub> | 165                |
| 21       | CH <sub>2</sub> —CH=CH <sub>2</sub> | (CH <sub>2</sub> ) <sub>2</sub> —S—(CH <sub>2</sub> ) <sub>3</sub> | 107                |
| 22       | C <sub>6</sub> H <sub>5</sub>       | (CH <sub>2</sub> ) <sub>2</sub> —S—(CH <sub>2</sub> ) <sub>3</sub> | 179                |
| 23       | NH <sub>2</sub>                     | (CH <sub>2</sub> ) <sub>2</sub> —S—(CH <sub>2</sub> ) <sub>3</sub> | 196                |

\* Decomposed.

55 The preparation of these compounds has been described in U.S. Pat. No. 3,647,451.



M.P. 197° C.



M.P. 195° C.

60 65 These compounds are prepared by reacting thiocarbo-

hydrazide with carbon disulfide in pyridine as described in *Acta Chemica Scandinavica* 15, pages 1295-1302 (1961). The compounds according to the invention may, of course, also be present in the corresponding thione form.

The concentration of the mercaptotriazole compounds in the image receiving layer may vary within wide limits. This depends on the requirements of the reproduction process and effectiveness of the particular compounds. Quantities of between 1 and 300 mg./m.<sup>2</sup> and preferably between 5 and 100 mg./m.<sup>2</sup> of image receiving layer, have generally been found to be sufficient. The triazole derivatives are soluble in aqueous alkalies or dimethylformamide and may be added in form of solution to the casting solutions for the production of the image receiving layer.

The image receiving material generally consists of an image receiving layer on a suitable support. The support may be the known sheet-like materials, particularly paper, preferably baryta-coated paper.

Suitable binders for the image receiving layer are the hydrophilic film-forming materials usually used for this purpose, e.g. proteins, particularly gelatin, also starch or starch derivatives, alginic acid or derivatives thereof such as salts, esters or amides, also carragenates or synthetic binders such as polyvinyl alcohol, polyvinyl pyrrolidone, partially saponified polyvinyl acetate, etc.

According to a preferred embodiment, the image receiving layer contains development nuclei of the usual type, e.g. sulfides or selenides of heavy metals such as cobalt, nickel, zinc or silver, and, furthermore nuclei of these metals. Modified nuclei of heavy metal sulfides or heavy metal selenides consisting of a core of an inert material, of a metal or of a sulfide or selenide other than that present in the surface, are also suitable. Nuclei of this type have been described in German Pat. No. 1,201,997 or in U.S. Pats. Nos. 2,698,236; 2,698,238 or 2,698,245.

The image receiving layers may, of course, contain the usual additives, particularly blue toners. Image receiving layers of this type have been described in German Pats. Nos. 1,108,563; 1,124,355; 1,124,354 and 1,153,247. The usual light-sensitive materials which generally contain a light-sensitive silver halide gelatin emulsion layer are suitable for the modification of the silver salt diffusion process according to the invention. The process is otherwise performed in the usual manner. Development may be carried out in a bath which contains developer or, in cases where the developer is present in the light-sensitive layer, a so-called activator solution which consists substantially of an aqueous alkaline bath may be used.

The materials may also be added to the developer bath or the activator bath such that they are taken up by the image receiving layer when the materials are being processed.

Quantities of 1 to 300 mg., preferably 50 to 250 mg./m.<sup>2</sup> are suitable in this case. When the materials are used in an activator, an additional advantageous effect is obtained in that the formation of dark silver sludge in the processing bath is reduced or becomes paler and, therefore, no longer gives rise to trouble.

#### EXAMPLE 1

##### Image receiving material

A baryta-coating of the following solution is applied to a support of paper (80 g. per m.<sup>2</sup>):

6 g. of a 50% aqueous suspension of barium sulfate, 20 ml. of a 10% aqueous gelatin solution, 8 ml. of a 50% aqueous emulsion of polyvinyl acetate,

(Water up to 100 ml.)

The baryta layer is dried and then coated with an image receiving layer of the following casting solution:

4.5 g. of propylene glycol alginate

12.5 mg. of silver sulfide in the form of an aqueous colloidal solution,

| Compound No.   | Concen-<br>tration,<br>g./l. | Maximum density |                                                |
|----------------|------------------------------|-----------------|------------------------------------------------|
|                |                              | Air dried       | After storage<br>in moist heat<br>for 24 hours |
| Control sample |                              | 1.20            | 0.91                                           |
| 2              | 0.5                          | 1.26            | 1.18                                           |
| 7              | 0.5                          | 1.27            | 1.15                                           |
| 9              | 0.5                          | 1.27            | 1.15                                           |
| 10             | 0.5                          | 1.27            | 1.23                                           |
| 16             | 0.25                         | 1.25            | 1.15                                           |
| 18             | 0.25                         | 1.30            | 1.19                                           |
| 20             | 0.5                          | 1.28            | 1.17                                           |
| 24             | 0.25                         | 1.27            | 1.16                                           |

Whereas the copies of the control sample are discolored brown to pale brown as a result of storage, the copies which contain the compounds according to the invention remain dark brown to blue-black. Moreover, the figures obtained with the air dried samples show that some of the

compounds according to the invention slightly accelerate the deposition of silver.

#### EXAMPLE 2

The light-sensitive silver halide layer contains about 600 mg. of hydroquinone and 150 g. of 1-phenylpyrazolone-(3) per m.<sup>2</sup>.

The light-sensitive layer is exposed, contacted with an image receiving layer as described in Example 1 and developed in the following activator solution instead of in the developer bath indicated in Example 1:

|                           | G.  |
|---------------------------|-----|
| Sodium sulfite sicc.      | 40  |
| Sodium phosphate sicc.    | 30  |
| Sodium hydroxide          | 1.5 |
| Sodium thiosulfate cryst. | 1   |
| Potassium bromide         | 1   |
| Water to up to 1 l.       |     |

After a contact time of 10 seconds they are separated. Subsequent processing and testing are carried out as described in Example 1. The quantities of the mercapto triazoles added to the image receiving layer are shown in the following Table:

| Compound No.   | Concen-<br>tration,<br>g./l. | Maximum density |                                                |
|----------------|------------------------------|-----------------|------------------------------------------------|
|                |                              | Air dried       | After storage<br>in moist heat<br>for 48 hours |
| Control sample |                              | 1.26            | 0.74                                           |
| 5              | 0.5                          | 1.25            | 1.16                                           |
| 6              | 0.5                          | 1.27            | 1.11                                           |
| 14             | 0.5                          | 1.30            | 1.07                                           |
| 15             | 0.5                          | 1.24            | 1.13                                           |
| 18             | 0.25                         | 1.30            | 1.14                                           |
| 19             | 0.5                          | 1.29            | 1.11                                           |
| 20             | 0.5                          | 1.27            | 1.19                                           |
| 22             | 0.25                         | 1.28            | 1.05                                           |
| 25             | 1.0                          | 1.24            | 1.08                                           |

Whereas the blacks of the control sample are discolored to pale brown in the course of storage, the copies containing the compound according to the invention remain dark brown to blue black.

#### EXAMPLE 3

190 mg. of compound 17 or 160 mg. of compound 15 are added per liter to an activator bath as described in Example 2. The material is then processed in a similar manner to the control sample in Example 1 or 2. Here again, a marked improvement in the loss in density on storage in moist heat is observed. When approximately 100 DIN A 4 copies are produced in 1 l. of activator, a sludge which gives it a very dark discoloration is formed in the activator which does not contain additive and the apparatus becomes severely soiled, whereas in the activators which contain additives a pale sludge is formed which is hardly visible and forms only a slight deposit on the walls of the apparatus.

We claim:

1. A light-insensitive image receiving material for the silver salt diffusion process comprising an image receiv-

60

ing layer which contains a compound of the following formula:



wherein

$\text{R}^1$ =a mercapto group or the group



$\text{R}^2$ =(I) an amino group (II) together with  $\text{R}^1$  the ring members required for completing a 2-mercaptop-thiadiazole ring or (III) in the case of a bis-triazole compound,  $\text{R}_2=\text{R}_3$ ;

$\text{R}^3$ =hydrogen, alkyl containing up to 8 C-atoms, aryl, aralkyl, cycloalkyl or an amino group;  $\text{Y}$ =an alkylene chain containing 3 to 10 methylene groups which are interrupted by oxygen, sulfur or imino groups.

2. A silver salt diffusion process in which an exposed recording material which contains at least one silver halide emulsion layer is developed in contact with an image receiving material in the presence of a heterocyclic mercapto compound of the following formula:



30 wherein

$\text{R}^1$ =a mercapto group or the group



$\text{R}^2$ =(I) an amino group (II) together with  $\text{R}^1$  the ring members required for completing a 2-mercaptop-thiadiazole ring or (III) in the case of a bis-triazole compound,  $\text{R}_2=\text{R}_3$ ;

$\text{R}^3$ =hydrogen, alkyl containing up to 8 C-atoms, aryl, aralkyl, cycloalkyl or an amino group;  $\text{Y}$ =an alkylene chain containing 3 to 10 methylene groups which are interrupted by oxygen, sulfur or imino groups.

#### References Cited

#### UNITED STATES PATENTS

3,438,777 4/1969 Wilrijk ----- 96-29  
2,514,650 7/1950 Knott ----- 95-7

NORMAN G. TORCHIN, Primary Examiner

J. L. GOODROW, Assistant Examiner

U.S. CL. X.R.

96-52

UNITED STATES PATENT OFFICE  
CERTIFICATE OF CORRECTION

Patent No. 3,674,481

Dated April 13, 1971

Inventor(s) James A. Pyne, Jr., et. al.

It is certified that error appears in the above-identified patent and that said Letters Patent are hereby corrected as shown below:

On the cover sheet, insert -- [73] Assignee The Garrett Corporation, Los Angeles, Calif., a corp. of California -- .

This certificate supersedes Certificate of Correction issued May 2, 1972.

Signed and sealed this 12th day of December 1972.

(SEAL)

Attest:

EDWARD M.FLETCHER,JR.  
Attesting Officer

ROBERT GOTTSCHALK  
Commissioner of Patents